

# United States Patent

Kambayashi et al.

[15] 3,656,942  
[45] Apr. 18, 1972

[54] STEEL FOR LOW-TEMPERATURE  
SERVICE

- [72] Inventors: Akira Kambayashi; Shun-Ichi Shimada, both of Kawasaki, Japan  
[73] Assignee: Nippon Kokan Kabushiki Kaisha, Kawasaki-shi, Kanagawa-ken, Japan  
[22] Filed: June 17, 1970  
[21] Appl. No.: 47,155

[30] Foreign Application Priority Data

- June 21, 1969 Japan.....44/48793  
[52] U.S. Cl. ....75/124, 75/123 B, 75/123 K,  
148/36  
[51] Int. Cl. ....C22c 39/02, C22c 39/36  
[58] Field of Search.....75/123 K, 123 L, 124, 123 B;  
148/36, 39

[56]

References Cited

UNITED STATES PATENTS

- 3,444,011 5/1969 Nagashima.....148/36 X  
3,496,034 2/1970 Alger .....148/36 X

Primary Examiner—L. Dewayne Rutledge

Assistant Examiner—J. E. Legru

Attorney—Flynn & Frishauf

[57]

ABSTRACT

A steel having excellent notch toughness, for service at low temperatures, which can be used in the normalized or hardened and tempered condition and which contains 0.4-0.13 percent Carbon, 0.15-0.30 percent Silicon, 0.30-0.90 percent Manganese, 8.50-9.50 percent Nickel, 0.020-0.060 percent Aluminum, 0.008-0.020 percent Nitrogen. Balance, Iron and incidental impurities.

12 Claims, No Drawings

## STEEL FOR LOW-TEMPERATURE SERVICE

This invention relates to a steel having excellent notch toughness at low temperatures and which can be used in the normalized or hardened and tempered conditions. More specifically, this invention relates to a steel containing 0.04 - 0.13 percent C, 0.15 - 0.30 percent Si, 0.30 - 0.90 percent Mn, 8.50 - 9.50 percent Ni, 0.020 - 0.060 percent Al, 0.008 - 0.020 percent N and up to 0.010 percent phosphorus, up to 0.010 percent sulphur and the balance iron and incidental impurities.

Steels of the above type are known generally to the art as ASTMA 353-67a and 553-67 steels, but these known types are not generally suitable for low temperature use under severe conditions because of their low notch strength. There is, however, a great demand for low temperature service steels and in order to satisfy that demand efforts have been made to improve the properties of this general class of steels. It is, therefore, an object of the present invention to provide an improved steel of the general ASTMA 353-67a or 553-67 type having improved properties, particularly at low temperatures.

It has been found, by one aspect of the invention, that the objects of the invention can be achieved by restricting the chemical composition of the general class of steel to a preferred range far narrower than the general range and also by introducing critical amounts of aluminum and nitrogen into the steel so that a desired amount of aluminum nitride may be precipitated. The preferred steel may then be used in the normalized or hardened and tempered conditions.

The upper limit of the aluminum content is set at 0.060 percent to avoid problems of inclusions and reduced purity of the steel. The lower limit is set at 0.02 percent because below this figure no useful deoxidation is achieved nor is the nitrogen completely taken up.

The nitrogen content is controlled between 0.020 percent and 0.008 percent. The upper limit being determined by the upper limit of the aluminum content and the lower limit being determined by the requirement for at least a minimum amount of aluminum nitride.

The invention will be described in more detail by reference to a specific example.

## EXAMPLE

A steel having a chemical composition as set out in Table I below, was rolled to a plate thickness of 15 mm. Two samples of the rolled steel were then normalized at 800° C and tempered at 575° C and another sample was heat treated by hardening at 800° C quenching in water and tempered at 575° C for 1 hour. Tensile and impact tests were carried out on both samples as set out in Table II. The tensile testing was conducted at room temperature and the impact testing was conducted at -196° C.

TABLE I

| Composition   | C    | Si   | Mn   | P     | S     | Ni   | Al    | N     |
|---------------|------|------|------|-------|-------|------|-------|-------|
| Contents----- | 0.06 | 0.21 | 0.40 | 0.010 | 0.008 | 9.22 | 0.045 | 0.013 |
| -----         | 0.05 | 0.18 | 0.42 | 0.001 | 0.005 | 9.20 | 0.043 | 0.015 |

TABLE II

| Plate thickness gauge (mm.) | Heat treatment                  | Yield point (kg./mm. <sup>2</sup> ) | Tensile test                             |                      | Impact test                    |                                  |
|-----------------------------|---------------------------------|-------------------------------------|------------------------------------------|----------------------|--------------------------------|----------------------------------|
|                             |                                 |                                     | Tensile strength (kg./mm. <sup>2</sup> ) | Elongation (percent) | vE 0° (kgm./cm. <sup>2</sup> ) | vE-196° (kgm./cm. <sup>2</sup> ) |
| 15-----                     | {Normalizing and tempering----- | 56                                  | 72                                       | 39                   | 24                             | 12                               |
|                             | {Hardening and tempering-----   | 69                                  | 76                                       | 37                   | 25                             | 23                               |
| 20-----                     | {Normalizing and tempering----- | 54                                  | 71                                       | 39                   | 28                             | 15                               |
|                             | {Hardening and tempering-----   | 67                                  | 74                                       | 38                   | 30                             | 28                               |

NOTE.—\* "vE 0°" denotes an impact value at 0° C. "vE": v stands for V notch notched on test piece. E stands for energy.

From the above example, it will be seen that the steel of the present invention has comparable tensile properties to the known steels for use at low temperatures. The carbon and manganese contents have been reduced and the tensile strength characteristic has been maintained because of the

strengthening effect obtained from the precipitation of aluminum nitride.

The reduced carbon and manganese contents and the aluminum nitride precipitation also contribute to the improved impact or notch toughness shown in the sample.

What is claimed is:

1. A steel for low temperature service consisting essentially of 0.04 - 0.13 percent carbon, 0.15 - 0.30 percent silicon, 0.30 - 0.90 percent manganese, 8.50 - 9.50 percent nickel, 0.020 - 0.060 percent aluminum, 0.008 - 0.020 percent nitrogen, up to about 0.010 percent phosphorus, up to 0.010 percent sulphur and the balance iron and incidental impurities.
2. A steel as claimed in claim 1 having a tensile strength of at least 72 Kg/mm<sup>2</sup> and an impact strength of at least 24 Kgm/cm<sup>2</sup> in the normalized and tempered condition.
3. A steel as claimed in claim 1 having a tensile strength of at least 71 Kg/mm<sup>2</sup> and an impact strength of at least 28 Kgm/cm<sup>2</sup> in the hardened and tempered condition.
4. A steel as claimed in claim 1 having a tensile strength of at least 74 Kg/mm<sup>2</sup> and an impact strength of at least 30 Kgm/cm<sup>2</sup> in the hardened and tempered condition.
5. A steel as claimed in claim 1 consisting essentially of 0.06 percent carbon, 0.21 percent silicon, 0.40 percent manganese, 0.010 percent phosphorus, 0.008 percent sulphur, 9.22 percent nickel, 0.045 percent aluminum, 0.013 percent nitrogen balance iron and incidental impurities.
6. A steel as claimed in claim 1 consisting essentially of 0.05 percent carbon, 0.18 percent silicon, 0.42 percent manganese, 0.011 percent phosphorus, 0.005 percent sulphur, 9.20 percent nickel, 0.043 percent aluminum, 0.015 percent nitrogen balance iron and incidental impurities.
7. A steel as claimed in claim 2 consisting essentially of 0.06 percent carbon, 0.21 percent silicon, 0.40 percent manganese, 0.010 percent phosphorus, 0.008 percent sulphur, 9.22 percent nickel, 0.045 percent aluminum, 0.013 percent nitrogen balance iron and incidental impurities.
8. A steel as claimed in claim 2 consisting essentially of 0.05 percent carbon, 0.18 percent silicon, 0.42 percent manganese, 0.011 percent phosphorus, 0.005 percent sulphur, 9.20 percent nickel, 0.043 percent aluminum, 0.015 percent nitrogen balance iron and incidental impurities.
9. A steel as claimed in claim 3 consisting essentially of 0.06 percent carbon, 0.21 percent silicon, 0.40 percent manganese, 0.010 percent phosphorus, 0.008 percent sulphur, 9.22 percent nickel, 0.045 percent aluminum, 0.013 percent nitrogen balance iron and incidental impurities.
10. A steel as claimed in claim 3 consisting essentially of 0.05 percent carbon, 0.18 percent silicon, 0.42 percent manganese, 0.011 percent phosphorus, 0.005 percent sulphur, 9.20 percent nickel, 0.043 percent aluminum, 0.015 percent nitrogen balance iron and incidental impurities.
11. A steel as claimed in claim 4 consisting essentially of 0.06 percent carbon, 0.21 percent silicon, 0.40 percent manganese, 0.010 percent phosphorus, 0.008 percent sulphur, 9.22 percent nickel, 0.045 percent aluminum, 0.013 percent nitrogen balance iron and incidental impurities.
12. A steel as claimed in claim 4 consisting essentially of

0.05 percent carbon, 0.18 percent silicon, 0.42 percent manganese, 0.011 percent phosphorus, 0.005 percent sulphur, 9.20 percent nickel, 0.043 percent aluminum, 0.015 percent nitrogen balance iron and incidental impurities.

\* \* \* \* \*

UNITED STATES PATENT OFFICE  
CERTIFICATE OF CORRECTION

Patent No. 3,656,942

Dated April 18, 1972

Inventor(s) AKIRA KAMBAYASHI et al

It is certified that error appears in the above-identified patent and that said Letters Patent are hereby corrected as shown below:

Column 1, Table 1 - Under "P", "0.001" should be "0.011".

Signed and sealed this 26th day of December 1972.

(SEAL)

Attest:

EDWARD M.FLETCHER,JR.  
Attesting Officer

ROBERT GOTTSCHALK  
Commissioner of Patents